

June 6, 1933.

G. C. PERRY

1,912,792

INDEX TAB

Filed Jan. 7, 1932

Fig. 1



Fig. 2



Fig. 3



Inventor:

Grover C. Perry,

By Cromwell, Freist. Warden

Attest.

## UNITED STATES PATENT OFFICE

GROVER C. PERRY, OF CHICAGO, ILLINOIS

## INDEX TAB

Application filed January 7, 1932. Serial No. 585,228.

The present invention relates to celluloid articles such as index tabs, label holders, and the like, and has particular reference to improvements by which the utility of such articles is considerably enhanced.

While my invention will be understood to have general application, it will be described with particular respect to a preferred embodiment, namely, index tabs or filing guides.

Heretofore the attaching portion of celluloid articles such as index tabs employing remoistening glue has generally comprised cloth, due to the impossibility of providing an adequate union between celluloid and glue. To secure celluloid tabs to ledger sheets, guides, and cards, for example, it has been necessary to resort to celluloid solvents, heat and pressure.

A principal object of the present invention is to provide celluloid articles such as index tabs and label holders having celluloid attaching portions capable of forming a stable union with remoistening glue.

Another object is to provide an index tab having transparent attaching portions.

Still another object is the construction of an index tab having stopping or alignment means which does not prevent the tab from being fully opened, for example, for remoistening the glue.

These and other objects will be apparent from the following description of a preferred form of my invention.

Fig. 1 is a side view of a tab embodying the features of my invention;

Fig. 2 is an end view of the tab shown in Fig. 1; and

Fig. 3 is a side view showing a tab having transparent attaching portions secured to a sheet of paper having printing beneath the attaching portion.

The tab shown in the drawing comprises substantially parallel projecting side portions 10 and 11 joined together along one edge by a spacing strip 12. Preferably these side portions are transparent celluloid forming a window channel which is adapted to receive a label insert containing appropriate information. In certain cases only one of

the side portions need be transparent, and in other instances it may be desirable to provide colored side portions.

Celluloid spacing strip 12 is preferably secured to the inner faces of the side portions as described in Patent, No. 1,510,243, issued to me September 30, 1924. That is, the parts are assembled in their final position and a brush coated with a celluloid solvent is passed in contact with the outer surfaces, whereby the celluloid solvent passes between the side portions and the spacing strip to form an intimate union. By employing appropriate colors these spacing strips may be used for signal purposes.

To the open edges of sides 10 and 11 are joined attaching portions 13 and 14, respectively. Ordinarily, the attaching portions will be joined to the inner faces of the sides as shown at 15 and 16 in Fig. 2, the joints being made permanent by welding with a celluloid solvent or cement.

Attaching portion 14 extends beyond portion 13 to facilitate insertion of a sheet to which it is desired to secure the tab. The upper edge of portion 14 may be turned over to form a hook 17. Being made of celluloid, which has considerable stiffness, this hook will retain its shape, where paper or cloth would not. This structure is of considerable utility since it forms a stop for sheets inserted between the attaching portions, thereby permitting the alignment of tabs in a uniform and satisfactory manner, and insures that the projecting sides or window portions will remain visible subsequent to attachment of the tab to a sheet. In addition, the member 17 is of particular utility in combination with my new celluloid attaching portions. More specifically, this type of stop member permits the tab to be fully opened so that the inner faces of the attaching portions may be easily moistened without stress or strain.

The attaching portions are composed of celluloid and are consequently less flexible than the cloth attaching portions of the prior art.

In the prior art many attempts have been made to solve the problem of attaching a water soluble or remoistening glue to celluloid,

but prior to my invention such efforts were without material success. Natural gums, pastes and glues do not adhere to celluloid as to paper, cloth, and the like. Apparently, 5 this is due to the non-porous character of the celluloid, and also to the lack of surface or specific adhesion between the molecules of glue and those of celluloid. Attempts have been made to dilute glue with a celluloid solvent, but the results of this procedure are unsatisfactory.

In accordance with my invention, the celluloid forming the attaching portion of the tab is coated with a solution similar to that 15 employed in the so-called "subbing" process of the photographic art. This solution may conform approximately to the following formula:

|    |                     |          |
|----|---------------------|----------|
| 20 | Water               | 1 part   |
|    | Glacial acetic acid | 9 parts  |
|    | Alcohol             | 90 parts |
|    | Gelatin             | 1 part   |

I have found that after a sheet of celluloid 25 treated with such a solution has dried, it affords an excellent base for a remoistening glue, whereby the celluloid may be employed for direct attachment to paper and the like. Thus, index tabs and other celluloid articles 30 having transparent attaching portions may be made of the material.

When the volatile portions of the above solution have evaporated, the surface of the celluloid is provided with a firmly held coating 35 of a glue adherent substance. An ordinary remoistening or water soluble glue is then applied to the celluloid at the portion having the glue adherent substance, and after drying the celluloid is ready for use. This 40 operation is preferably done with sheets of celluloid before the sheets have been formed into the desired article.

From the foregoing description, it is seen 45 that in accordance with my invention I provide a tab with celluloid fastening portions having all the utility of the ordinary cloth attaching portions. Also the tab may be attached to a sheet having printed matter adjacent the edges thereof, without rendering such matter illegible. The transparency of 50 the attaching portion permits printed matter, marks, and the like to be readily observed therethrough, as shown in Fig. 3.

It is to be understood that the above 55 description of a preferred modification is for the purposes of explanation and illustration, and that the many modifications coming within the spirit of my invention are intended to be covered by the appended claims. For 60 example, the term "celluloid" as used in the specification and claims is intended to cover the product known as celluloid and other plastic substances of like character.

I claim:

65 1. A tab, comprising substantially parallel

window portions composed of transparent celluloid, a spacing strip joining said window portions along one side, transparent celluloid attaching portions joined to the inner faces of said window portions along the opposite side thereof and provided with a glue adherent substance.

70 2. A tab, comprising substantially parallel window portions composed of celluloid and joined at one side, and celluloid attaching portions joined to the inner faces of said window portions along the opposite side thereof and provided with a glue adherent substance, the joining edge of one of said attaching portions being turned over to form 75 a stop.

3. A tab, comprising substantially parallel sides, and separate attaching portions joined to the inner faces of said sides, one of said portions being turned over to form a stop.

80 4. A tab, comprising a celluloid window portion, and a celluloid attaching portion secured to the inner face of said window portion, said attaching portion having its upper edge turned over to form a stop.

85 5. A tab having a celluloid attaching portion coated with a glue adherent, gelatine, and a coating of remoistening glue covering said gelatine.

90 6. The method which comprises coating celluloid with a celluloid solvent and a glue adherent gelatine, drying said celluloid, and applying thereto a remoistening glue.

95 7. The method of forming a tab, which comprises assembling strips of celluloid in 100 spaced parallel relation, uniting corresponding edges of said strips to form one end of the tab, coating the inner faces of said strips with a solution containing a celluloid solvent and a glue-adherent gelatin, and coating said 105 gelatin with a remoistening glue.

110 In testimony whereof I have hereunto subscribed my name.

GROVER C. PERRY.

110

115

120

125

130